

## UNITED STATES PATENT OFFICE

2,364,284

## MODIFIED LUBRICATING OIL

Herbert C. Freuler, Orinda, Calif., assignor to  
 Union Oil Company of California, Los Angeles,  
 Calif., a corporation of California

No Drawing. Application June 17, 1941,  
 Serial No. 398,459

38 Claims. (Cl. 252—39)

This invention relates principally to lubricating oils, but may be extended also to other forms of lubricants such as greases, the so-called liquid greases and the like. The object of the invention is to produce lubricating oils and other lubricants having high film strength, good oiliness characteristics, resistance to oxidation and to corrosion as by inhibiting the development of oxidation and corrosive conditions in the lubricants.

This application is a continuation-in-part of my prior application Serial No. 156,946, filed August 2, 1937.

I have discovered that by the addition of minor proportions of oil-soluble metal salts of alkyl esters of thio acids of phosphorus to lubricating oils, with or without the addition of other agents to the oils such as soaps and the like for the purpose of imparting detergent properties or thickening the oils, the resistance of oils to oxidation is greatly improved by what appears to be an inhibiting action on the part of the metal salts of the thiophosphates. Also the tendency to corrosion of metals by reason of the presence of some types of addition agents introduced into compounded oils to impart extreme pressure characteristics, is inhibited by these metallic derivatives of the phosphorus acids. This may apply to lubrication of gears, internal combustion engines, and other metal parts. Also the mentioned phosphates exert an inhibiting action against the development of conditions which are corrosive to highly corrosion-sensitive bearings in internal combustion engines and the like, such as Diesel engines and high-output aviation engines. For example, some highly refined lubricating oils have a tendency toward the development, apparently by oxidation, of acids corrosive to bearings such as cadmium-silver and copper-lead bearings while in use in internal combustion engines. Also similar corrosive acids tend to develop in some compounded oils while in use. Examples are oils which contain various detergent soaps now used in Diesel engines and the like. These soaps normally are added to the oils to overcome valve and ring sticking and the like and to keep the pistons and ring grooves clean. Such soaps include the oil-soluble metal soaps of various carboxylic acids such as chlorinated and phenylated fatty acids, oil-soluble metal soaps of high molecular weight acids derived from the oxidation of highly paraffinic petroleum fractions such as highly refined lubricating oils, and the like. These soaps, which may be alkaline earth metal soaps or heavy metal

soaps such as calcium, magnesium, barium, zinc, lead, manganese and aluminum soaps, tend to catalyze oxidation with the formation of acids, possibly carboxylic acids, which are corrosive to the mentioned highly corrosion-sensitive copper-lead and cadmium-silver type.

I have found that by employing minor proportions of the metal phosphates of the present invention with these various oils or compounded 10 oils, the tendency toward oxidation and the development of the corrosive conditions is materially inhibited. For example, I may employ in the order of from  $\frac{1}{2}\%$  to 2.0% of various detergent soaps in an oil, and inhibit corrosion otherwise resulting from such soaps, by employing from 0.1% to 1.0% or 2.0% of one of the present 15 metal thiophosphates as an inhibitor. These salts may also be added to compounded oils other than those mentioned. Again, I may add corresponding proportions of one of these metal thiophosphates to a highly refined highly paraffinic mineral lubricating oil and similarly inhibit oxidation and the development of corrosive conditions. This control of corrosion may or may not 20 be the same type of control as that resulting where chlorinated or sulfurized extreme pressure agents are added to lubricants. Similarly I may use the corresponding metal phosphates which have no sulfur content and are wholly 25 of the oxy-phosphate type, to control oxidation and corrosion.

My invention therefore resides primarily in the employment in compounded or in uncompounded mineral lubricating oils, of minor proportions of 30 oil-soluble metal salts of the thio acids of phosphorus substituted with organic radicals such as alkyl radicals which tend to render the salt oil-soluble. In addition to alkyl groups, other organic substituents of sufficiently high molecular 35 weight to render the salts oil-soluble may be employed, such as aryl radicals, alkaryl radicals and the like. Other suitable metals are the alkaline earth metals, calcium, magnesium and barium, and the lighter of the so-called "heavy 40 metals" such as zinc and aluminum, and other "heavy metals" such as lead, mercury, copper, manganese, iron, tin, bismuth, and thorium. For example, for the purpose of producing a most desirable extreme pressure agent I have employed 45 zinc salts of octyl and di-octyl thiophosphates, and on an average about 1.0% thereof based on the oil in the case of lubricating oils, or total content if a grease, has been found very satisfactory. Other alkyls may be employed as substituents, particularly the heavier ones inasmuch as these 50

render the salts oil-soluble. Examples are the heptyl, decyl, dodecyl or lauryl, oleyl and similar alkyl groups.

The corresponding or similar metal phosphates free from sulfur, i.e., wholly oxy-phosphates, are also included in the invention as anti-oxidants and the like.

Salts of these produced from the various metals indicated are good inhibitors of oxidation and of corrosive conditions otherwise developed while in use, and are good inhibitors or retarders of corrosive conditions which result from the use of corrosive oiliness agents and the like containing halogens and corrosive sulfur, for example. The zinc salts have been found very desirable in the preparation of extreme pressure agents, and calcium and barium salts are very desirable as oxidation and corrosion retarders.

Instead of alkyl groups as solubilizing constituents phenyl groups, alkylated phenyl groups, naphthalene and anthracene groups may be employed, together with kindred aryl groups and alkylated aryl groups, such as amyl-substituted phenol groups or octyl-substituted phenol or naphthyl groups, or cresyl groups.

A specific example of this invention which is particularly valuable as a high film strength and oiliness agent, and which also imparts some oxidation inhibiting value to oils compounded therewith, is zinc di-octyl thiophosphate. The corresponding lead salt is also useful. When zinc octyl thiophosphate (produced from zinc oxide and the reaction product of octyl alcohol and phosphorus pentasulfide as herein described) was used in an amount approximating 1.0% as an addition agent to lubricating oils, the load which the oil was capable of withstanding when tested by the well known Timken Lubricant tester at 800 R. P. M. (described in S. A. E. Journal, vol. 28, 1931, pages 53-60) was increased from seven pounds without the agent to forty-five pounds when employing the agent. In addition to this film strength increase, the oil is made much more resistant to oxidation than in its original state. Moreover, the metallic salts of the alkyl thiophosphates in proportions here indicated inhibit, to a marked degree, the corrosion of metals by oils which contain sulfur, chlorine, corrosive sulfur compounds, corrosive halogenated bodies, or corrosive organic compounds containing sulfur or halogen. Where these corrosive materials are present in relatively large amounts somewhat more than 1.0% of alkyl thiophosphate may be used as necessary or desirable in accomplishing the desired end. In addition to the use of lead or zinc octyl thiophosphate, other metal salts may be employed, and likewise other alkyl thiophosphates of such metals may be used. Examples of such other metals are aluminum, calcium, magnesium and others herein indicated.

In referring to the content of 1.0% of the salt in the lubricating oil, it is not intended to convey the idea that this amount is critical. Varying proportions may be employed in mineral lubricating oils between any lower range sufficient to produce the desired increased film strength, or oxidation control, for example, 0.1%, up to a figure such as 20% beyond which added material produces no appreciable increased effect. For example, 10% of lead or zinc dioctyl thiophosphate in an appropriate mineral oil, produces a very valuable hypoid gear lubricant. Blends containing about one percent of the salt entirely inhibit the corrosion which normally takes place upon copper and steel when strips

thereof are immersed in the lubricant for sixteen hours at 180° F. with water present and in contact with the strips.

As an example of the preparation of the alkyl thiophosphates, octyl thiophosphate has been prepared readily by adding powdered phosphorus pentasulfide to octyl alcohol in a glass or ceramic container in the proportion of one gram mol to four gram mols, respectively, and agitating the mixture at temperatures of 250° F. to 300° F. until the phosphorus pentasulfide has been dissolved. This liquid product is then treated at similar temperatures with an excess of a powdered metal or metallic oxide to form the corresponding metal derivative. For example, in order to prepare the zinc octyl thiophosphate, the material resulting from the treatment of octyl alcohol with phosphorus pentasulfide is agitated with powdered zinc or zinc oxide until no more of the metallic compound is dissolved. Similar preparations can be made with other metals, although in most cases it is preferable to use the metallic oxide. The metallic derivatives of octyl thiophosphate and similar thiophosphates are easily soluble in mineral oils of both western and eastern types (naphthenic and paraffinic) and the oil solutions are therefore readily prepared by mere introduction of the salt and subsequent mild agitation. The term "octyl thiophosphate" used in this disclosure may refer to either the di- or the mono-octyl thiophosphate, although it is the di-octyl thiophosphate which is the principal product of the above preparation. This is usually true of the other phosphates.

The specific material produced by the method above described showed rapid reaction with evolution of hydrogen sulfide when the temperature reached 250° F. The phosphorus pentasulfide had all gone into solution, that is had entered into chemical combination, in about two hours. This material analyzed 18.1% sulfur and 9.3% phosphorus. This indicated a product of the following composition:



There is some evidence of the presence of a mono-octyl thiophosphate which would have the formula:



Other possible combinations are:



The product produced as above described may be a mixture of all of these esters. In any event the mixture contains the oxy-esters of the thio acid of phosphorus as shown in the first formula. This is well established by the authorities on the chemistry of this reaction and is clearly supported by the analysis of the compound produced. Also, this may be considered as the dioctyl ester of an oxy-thio-acid of phosphorus.

Again there may be present what may be termed a thio ester of an oxy-acid of phosphorus,

or an oxy-thio-acid of phosphorus. Such a material could have the formula:



This can also be considered any oxy-thio-ester or an ester of an oxy or oxy-thio acid of phosphorus.

While the octyl phosphates are particularly mentioned above, the  $C_8H_{17}$  group may be replaced in each formula with another alkyl group such as decyl or other organic radical herein described, such as indicated by R in the following as an example:



The metal salts of these thiophosphates produced by the method above described were prepared by mixing the described ester with an excess of the oxides of the respective metals, such as zinc, lead, copper, manganese, iron and tin, and allowing the resultant mixtures to stand overnight at about 250° F. Upon decanting and filtering, light colored viscous liquids were obtained except in the case of iron and manganese where the liquids were dark.

These various metal salts of the thiophosphate esters were blended in a highly solvent refined highly paraffinic western lubricating oil in the amount of about 1.0% of the ester to 99% of the oil, and tested on the well known Timken tester for extreme pressure characteristics. In each instance an increase in the film strength was noted as measured by the increase in load supported over that supported by the same oil untreated. Similar results were obtained by testing each of the materials in the same proportion in the same oil upon the S. A. E. extreme pressure lubricants tester.

Each of the above described blends was also subjected to a corrosion test and found to show definite inhibition of corrosion to metals, although some exhibited greater corrosion inhibiting properties than others. Similarly each blend was tested and found to possess distinct oxidation inhibiting properties in the oil.

As an example of the salts, i. e., the phosphates, and the preparation of such metal phosphates which are wholly oxy-phosphates and free from sulfur, the following is given. Octyl alcohol is reacted with powdered phosphorus pentoxide ( $P_2O_5$ ) in a glass or ceramic container in suitable mol proportions under conditions similar to those above described for the preparation of the thiophosphates. The liquid product obtained is similarly treated with an excess of the powdered metal or metallic oxide required for the desired metal derivative. Other aliphatic alcohols within the range herein indicated may be produced in a similar manner using phosphorus pentoxide. By this procedure metal salts of substituted oxy acids of phosphorus are produced which correspond with the thio-phosphates previously described.

For production of either the thio-phosphates or the oxy-phosphates, the method may be such as that disclosed by the Christmann Patent 1,893,018 for making thio-phosphates using  $P_2S_5$ .  $P_2O_5$  may be substituted for the  $P_2S_5$  in making the oxy-phosphates.

The oxy-phosphates may be prepared from the

various substituted oxy-acids of pentavalent phosphorus of the following and similar types:



wherein R and R' will be alkyl, aryl, alk-aryl or ar-alkyl groups such as previously indicated which are sufficiently heavy in carbon atoms to render the eventual salts sufficiently oil-soluble. R and R' may be the same or different groups.

These substituted oxy-acids of phosphorus may be prepared by any of the various methods known in the art. For example the method of the Graves Patent 2,005,619 using phosphorus oxy-chloride ( $POCl_3$ ) may be employed. Here the alcohol, with or without a solvent such as benzene, is heated in an acid-resistant vessel with a reflux

20 condenser at reduced pressure to a temperature in the order of 30° C., or from 0° C. to 100° C., and the phosphorus oxy-chloride is gradually introduced in liquid or vapor form, the liberated hydrogen chloride being largely removed as

25 formed. For the present purpose I may use the esters, or mixed esters, or mixtures of esters of the various acids of phosphorus, namely ortho-phosphoric acid, meta-phosphoric acid, pyro-phosphoric acid, phosphorous acid, and hypo-phosphorous acid, as disclosed by Graves. Oil-soluble metal salts of these esters may be prepared in any suitable manner such as indicated herein. Thus I may use oil-soluble di-octyl phosphate of one of the alkaline earth metals, or the di-decyl phosphate, or an oil-soluble alkaline earth metal octyl-decyl phosphate, such as the ortho-phosphate.

In general the alkyl groups employed will contain from around eight to around twenty carbons per molecule to insure sufficient oil-solubility. Again the aromatic or ring compounds may be employed, these being used in sufficient number per molecule, or in form modified by an alkyl, to insure oil-solubility.

40 45 According to another method for the preparation of the substituted oxy-acids of phosphorus, a mixture of an alcohol of the required type (higher alcohol) such as octyl alcohol, or phenol, or cresol, or alkylated phenol, with phosphorus pentoxide in ethyl ether is refluxed for several hours. This produces an alkyl-phosphoric acid which is soluble in the ether. The ether solution is decanted from any insolubles and the alkyl-phosphoric acid recovered. Where the ethyl group enters into the alkyl-phosphoric acid it may be eliminated by hydrolysis.

50 55 Appropriate metal salts of the various substituted oxy-acids of phosphorus thus obtained may be conveniently prepared by reacting the acid with sodium or potassium hydroxide, and then precipitating the desired metal salt from the solution by the addition of a suitable metal compound such as a calcium salt or aluminum salt. Also, the desired phosphate may be prepared 60 from the substituted oxy-acids by direct neutralization, for example, with zinc oxide or with lime, according to the salt finally desired. Salts of the alkaline earth metals, calcium, barium, strontium, lithium and magnesium, are valuable, as are those of zinc, lead, chromium, bismuth, thorium, aluminum, copper, iron, tin, manganese and the like herein mentioned.

The various salts so prepared from the substituted oxy-acids as just given and the various 65 70 75 thio-salts previously described are adequately sol-

uble in mineral lubricating oils, and are used according to this invention to control the sticking of piston rings and the like and also to control other oxidation effects and tendencies to develop corrosive conditions in lubricating oils when used in internal combustion engines and the like, especially severe service engines such as Diesel engines. Calcium and zinc dioctyl phosphates and oleyl and lauryl phosphates are good examples.

The proportions of the salts both of the straight oxy-materials free from sulfur and of the thio-materials used in lubricating oils will be similar and in the order of those previously indicated. For example around 1.0% probably will be commonly used although proportions between about 0.5% and 2.0% will be in order and possibly for some uses as low as 0.1% or 0.2% or perhaps as high as 3% or 4%.

With respect to the various salts herein disclosed as additives for lubricating oils, possibly the alkaline earth metal salts are somewhat preferable to the other salts as anti-oxidants or corrosion inhibitors, and the salts of the other metals are possibly preferable as extreme pressure agents.

I claim:

1. A composition of matter comprising a hydrocarbon oil subject to deterioration at elevated temperature, and an alkaline earth metal salt of a sulfur-containing substituted acid of phosphorus having an organic substituent therein, said salt being present in an amount sufficient substantially to inhibit said deterioration.

2. A composition of matter comprising a hydrocarbon oil subject to deterioration at elevated temperature, and a calcium salt of a sulfur-containing substituted acid of phosphorus having an organic substituent therein, said salt being present in an amount sufficient substantially to inhibit said deterioration.

3. A composition of matter comprising a hydrocarbon oil subject to deterioration at elevated temperature, and a magnesium salt of a sulfur-containing substituted acid of phosphorus having an organic substituent therein, said salt being present in an amount sufficient substantially to inhibit said deterioration.

4. A composition of matter comprising a hydrocarbon oil subject to deterioration at elevated temperature, and an alkaline earth metal salt of a sulfur-containing substituted acid of pentavalent phosphorus having an organic substituent therein, said salt being present in an amount sufficient substantially to inhibit said deterioration.

5. A composition of matter comprising a hydrocarbon oil subject to deterioration at elevated temperature, and a calcium salt of a sulfur-containing substituted acid of pentavalent phosphorus having an organic substituent therein, said salt being present in an amount sufficient substantially to inhibit said deterioration.

6. A composition of matter comprising a hydrocarbon oil subject to deterioration at elevated temperature, and a magnesium salt of a sulfur-containing substituted acid of pentavalent phosphorus having an organic substituent therein, said salt being present in an amount sufficient substantially to inhibit said deterioration.

7. A stabilized liquid lubricant comprising a lubricating oil and an alkaline earth metal salt of a sulfur-containing substituted acid of phosphorus having an organic substituent therein, said salt being present in an amount sufficient

substantially to stabilize said oil against deterioration during use.

8. A stabilized liquid lubricant comprising a lubricating oil and an alkaline earth metal salt of a sulfur-containing substituted acid of pentavalent phosphorus having an organic substituent therein, said salt being present in an amount sufficient substantially to stabilize said oil against deterioration during use.

10. 9. A composition of matter comprising a hydrocarbon oil subject to deterioration in the presence of oxygen, and an alkaline earth metal salt of a thio-ester of phosphoric acid, said salt being present in an amount sufficient substantially to inhibit said deterioration.

10. 10. A composition of matter comprising a hydrocarbon oil subject to deterioration in the presence of oxygen, and a calcium salt of a thio-ester of phosphoric acid, said salt being present in an amount sufficient substantially to inhibit said deterioration.

11. A composition of matter comprising a hydrocarbon oil subject to deterioration in the presence of oxygen, and a magnesium salt of a thio-ester of phosphoric acid, said salt being present in an amount sufficient substantially to inhibit said deterioration.

12. A composition of matter comprising a hydrocarbon oil subject to deterioration in the presence of oxygen, and an alkaline earth metal salt of an ester of a thiophosphoric acid, said salt being present in an amount sufficient substantially to inhibit said deterioration.

13. A composition of matter comprising a hydrocarbon oil subject to deterioration in the presence of oxygen, and a calcium salt of an ester of a thiophosphoric acid, said salt being present in an amount sufficient substantially to inhibit said deterioration.

14. A composition of matter comprising a hydrocarbon oil subject to deterioration in the presence of oxygen, and a magnesium salt of an ester of a thiophosphoric acid, said salt being present in an amount sufficient substantially to inhibit said deterioration.

15. A composition of matter comprising a hydrocarbon oil subject to deterioration in the presence of oxygen and an alkaline earth metal salt of a thio-ester of a thio-phosphoric acid, said salt being present in an amount sufficient substantially to inhibit said deterioration.

16. A composition of matter comprising a hydrocarbon oil subject to deterioration in the presence of oxygen and a calcium salt of a thio-ester of a thiophosphoric acid, said salt being present in an amount sufficient substantially to inhibit said deterioration.

17. A composition of matter comprising a hydrocarbon oil subject to deterioration in the presence of oxygen and a magnesium salt of a thio-ester of a thiophosphoric acid, said salt being present in an amount sufficient substantially to inhibit said deterioration.

18. A stabilized liquid lubricant comprising a paraffinic lubricating oil subject to deterioration at elevated temperature and more than approximately 0.1% by weight based on the oil of a magnesium salt of a sulfur containing substituted acid of phosphorus having an organic substituent therein in an amount sufficient substantially to inhibit said deterioration.

19. A stabilized liquid lubricant comprising a paraffinic lubricating oil subject to deterioration at elevated temperature and more than approxi-

mately 0.1% by weight based on the oil of an alkaline earth metal salt of a sulfur-containing substituted acid of phosphorus having an organic substituent therein in an amount sufficient substantially to inhibit said deterioration.

20. A stabilized liquid lubricant comprising a paraffinic lubricating oil subject to deterioration at elevated temperature and more than approximately 0.1% by weight based on the oil of a calcium salt of a sulfur-containing substituted acid of phosphorus having an organic substituent therein in an amount sufficient substantially to inhibit said deterioration.

21. A composition of matter comprising a hydrocarbon oil subject to deterioration at elevated temperature and an alkaline earth metal salt of a sulfur containing substituted acid of phosphorus having an organic substituent of 8 carbon atoms therein, said salt being present in an amount sufficient substantially to inhibit said deterioration.

22. A composition of matter comprising a hydrocarbon oil subject to deterioration at elevated temperature and a calcium salt of a sulfur containing substituted acid of phosphorus having an organic substituent of 8 carbon atoms therein in an amount sufficient substantially to inhibit said deterioration.

23. A composition of matter comprising a hydrocarbon oil subject to deterioration at elevated temperature and a magnesium salt of a sulfur containing substituted acid of phosphorus having an organic substituent of 8 carbon atoms therein in an amount sufficient substantially to inhibit said deterioration.

24. A stabilized liquid lubricant comprising a lubricating oil subject to deterioration at elevated temperature and more than approximately 0.10% by weight based on the oil of an alkaline earth metal salt of a sulfur containing substituted acid of phosphorus having at least one organic substituent of 8 carbon atoms therein in an amount sufficient substantially to inhibit said deterioration.

25. A composition comprising a hydrocarbon oil subject to deterioration at elevated temperatures and an oil-soluble alkaline earth metal salt of an octyl thiophosphate, said salt being present in an amount sufficient substantially to inhibit said deterioration.

26. A composition of matter comprising a hydrocarbon oil subject to deterioration at elevated temperatures and an alkaline earth metal salt of a sulfur containing substituted acid of pentavalent phosphorus having two organic substituents therein, said salt being present in an amount sufficient substantially to inhibit said deterioration.

27. A composition of matter comprising a hydrocarbon oil subject to deterioration at elevated temperature and a calcium salt of a sulfur containing substituted acid of pentavalent phosphorus having an organic substituent therein in an amount sufficient substantially to inhibit said deterioration.

28. A composition of matter comprising a hydrocarbon oil subject to deterioration at elevated temperature and a magnesium salt of a sulfur containing substituted acid of pentavalent phosphorus having two organic substituents therein in an amount sufficient substantially to inhibit said deterioration.

29. A composition comprising a hydrocarbon oil

subject to deterioration at elevated temperatures and an oil-soluble alkaline earth metal salt of a di-octyl thiophosphate, said salt being present in an amount sufficient substantially to inhibit said deterioration.

30. A compounded lubricant comprising a lubricating oil subject to deterioration at elevated temperature and an alkaline earth metal salt of a sulfur-containing substituted acid of pentavalent phosphorus having more than approximately twelve carbon atoms in the molecule in an amount sufficient substantially to inhibit said deterioration.

31. A compounded lubricant comprising a lubricating oil subject to deterioration at elevated temperature and from approximately 0.1% to approximately 2% by weight based on the oil of a calcium salt of a sulfur-containing substituted acid of pentavalent phosphorus having more than approximately twelve carbon atoms in the molecule in an amount sufficient substantially to inhibit said deterioration.

32. A compounded lubricant comprising a lubricating oil subject to deterioration at elevated temperature and from approximately 0.1% to approximately 2% by weight based on the oil of a magnesium salt of a sulfur-containing substituted acid of pentavalent phosphorus having more than approximately twelve carbon atoms in the molecule in an amount sufficient substantially to inhibit said deterioration.

33. A lubricating oil containing a constituent corrosive to metal of the class consisting of sulfur, chlorine, sulfurized bodies, halogenated compounds, and metal corrosive organic compounds containing sulfur and halogens, and an oil-soluble alkaline earth metal salt of a sulfur containing substituted acid of phosphorus having an organic substituent therein, said salt being present in an amount sufficient to reduce oxidation and corrosion.

34. A composition of matter as claimed in claim 4, in which the sulfur containing substituted acid of pentavalent phosphorus having an organic substituent employed to produce the alkaline earth metal salt is obtained by reacting phosphorus pentasulfide with an alcohol.

35. A composition of matter as claimed in claim 5, in which the sulfur containing substituted acid of pentavalent phosphorus having an organic substituent employed to produce the calcium salt is obtained by reacting phosphorus pentasulfide with an alcohol.

36. A composition of matter as claimed in claim 6, in which the sulfur containing substituted acid of pentavalent phosphorus having an organic substituent employed to produce the magnesium salt is obtained by reacting phosphorus pentasulfide with an alcohol.

37. A composition of matter as claimed in claim 4, in which the sulfur containing substituted acid of pentavalent phosphorus having an organic substituent employed to produce the alkaline earth metal salt is obtained by reacting phosphorus pentasulfide with an aliphatic alcohol.

38. A composition of matter as claimed in claim 4, in which the sulfur containing substituted acid of pentavalent phosphorus having an organic substituent employed to produce the alkaline earth metal salt is obtained by reacting phosphorus pentasulfide with an octyl alcohol.

HERBERT C. FREULER.

6

CERTIFICATE OF CORRECTION.

Patent No. 2,364,284.

December 5, 1944.

HERBERT C. FREULER.

It is hereby certified that error appears in the printed specification of the above numbered patent requiring correction as follows: Page 1, first column, line 40, for "intenal" read --internal--; page 3, first column, line 7, for "any" read --an--; page 5, first column, line 63, claim 27, for "an organic substituent" read --two organic substituents--; and that the said Letters Patent should be read with this correction therein that the same may conform to the record of the case in the Patent Office.

Signed, and sealed this 20th day of March, A. D. 1945.

(Seal)

Leslie Frazer  
Acting Commissioner of Patents.